

M. M. MERRITT.  
GALVANOPLASTIC PROCESS AND PRODUCT.  
APPLICATION FILED DEC. 8, 1917.

1,321,793.

Patented Nov. 11, 1919.



Invensor:  
Matthew M. Merritt.  
by Emery Booth Jones, Verna  
Heiss.

# UNITED STATES PATENT OFFICE.

MATTHEW M. MERRITT, OF SOUTH MIDDLETON, MASSACHUSETTS, ASSIGNOR TO COPPER PRODUCTS COMPANY, OF BOSTON, MASSACHUSETTS, A CORPORATION OF MAINE.

## GALVANOPLASTIC PROCESS AND PRODUCT.

1,321,793.

Specification of Letters Patent. Patented Nov. 11, 1919.

Original application filed November 2, 1917, Serial No. 199,811. Divided and this application filed December 8, 1917. Serial No. 206,295.

*To all whom it may concern:*

Be it known that I, MATTHEW M. MERRITT, a citizen of the United States, and a resident of South Middleton, county of Essex, 5 5 Commonwealth of Massachusetts, have invented an Improvement in Galvanoplastic Processes and Products, of which the following description, in connection with the accompanying drawings, is a specification, 10 like characters on the drawings representing like parts.

This invention pertains to improvements in galvanoplastic processes and products, but more particularly, though not exclusively, 15 to the manufacture of articles such as manifolds for internal combustion engines such as aeroplane engines.

This application is a divisional of my co-pending application, Serial No. 199,811, filed 20 November 2, 1917.

In the drawings, which show one form of an illustrative embodiment of my invention:

Figure 1 shows a manifold; 25 Fig. 2 is a diagrammatic section therethrough on the line 2—2 of Fig. 1.

Great difficulty has been experienced in constructing manifolds for aeroplane engines of the requisite light weight which are 30 strong enough to withstand the constant and excessive vibrations occasioned by the operation of the engine. Such manifolds are very likely to develop cracks, particularly adjacent the bent portions thereof. It has 35 heretofore been attempted to manufacture such manifolds by the electrolytic deposit of copper on cathodes of metal fusible at a low temperature, and on cathodes of wax painted with graphite or other electrically conductive material, the core being melted out 40 after the electrolyte deposit. Manifolds made by the usual methods, above-described, have proved unsatisfactory because of brittleness and coarseness of texture of the deposited metal, this brittleness being accentuated 45 at points adjacent curved portions of the deposit.

I have found that the deposits made as before described are rendered more uniform 50 in quality by intermittent immersion of the cathode, as by attaching the same to a revolving wheel partially immersed in the electrolyte so that the entire cathode or a

considerable portion thereof, preferably at least one-half, is only intermittently immersed in the electrolyte. While intermittent immersion improves the texture of the deposited metal, electrolytic deposits made on metallic cathodes having low melting points are, as heretofore made, likely to be 55 rough and brittle. I believe this to be due to the tendency of certain ingredients of the fusible metal, which is usually an alloy of lead, to be attacked by the electrolyte, and in some instances to be disassociated into 60 negative ions traveling from the cathode to the anode.

Where, on the other hand, the cathode is formed of non-conductive material removable by fusion, by a solvent, or otherwise, 70 and the surface of which is coated with an electrically conductive paint, such as graphite, bronze powder and the like, the deposited copper, as heretofore practised, has been brittle and of slight tensile strength. 75 As stated in my co-pending application, filed herewith, I believe this to be due to the comparatively coarse texture of the conductive coating which is necessarily full of interstices as compared with cast, rolled, or 80 electrolytically deposited metal. The unevenness of attraction exerted by this surfacing of the cathode results in combining the deposited metal in relatively coarse crystalline formation, which renders it brittle and 85 of slight tensile strength.

I have found that the deleterious effects of a cathode composed of metal having a low fusing-point may be minimized by coating the metal with a film of a foreign substance such as grease, and that if a layer of copper, preferably relatively thin, be electrolytically deposited subsequent to the application of the grease and the surface of this metal be coated with grease, that subsequent electrolytic deposits on the greased surface will be of fine texture and of great tensile strength, the brittleness being greatly reduced, if not eliminated. If desired, the structure may be laminated by the occasional 90 interruption of electrolytic deposit and the application to the surface of the deposited metal of films of grease.

Where it is necessary or desirable to utilize a non-metallic cathode such as wax 105 or any electrically non-conductive material

removable by a solvent or otherwise, the same being coated with a paint of electrolytically conductive material, I have found it of great advantage to coat the surface of 5 the electrically conductive material or paint with a thin film of grease, to deposit a relatively thin sheet of copper or other metal on the greased surface and, if desired, to provide a laminated structure by subsequently 10 occasionally interrupting the electrolytic deposit and applying grease to the surface of the deposited metal.

Throughout this application I have used 15 the word "grease" generically to define any substance capable of forming a film of electrically non-conductive material over the surface on which metal is to be deposited.

After electro-deposition the core of the cathode may be removed by fusion, by burning, by the use of a solvent or any other 20 suitable method.

I have utilized the word "galvanoplastic" 25 in its broader sense to include any electrolytic processes in which the entire cathode or any portion thereof is removed subsequent to electro-deposition.

It is obvious that the cathode may, if desired, be exterior to the surface thereof on 30 which metal is to be deposited, and that for some purposes my invention may be useful in connection with galvanoplastic processes

in which the cathode can be withdrawn without change in the structure thereof.

While I have shown and described one embodiment of my invention and one 35 method of practising the same, it will be understood that major changes may be made, both in the product and the method of producing the same, without departing from the scope of my invention, which is 40 best defined in the following claims:

1. The galvanoplastic process which comprises coating a mold or core with a coating of electrically conductive granular material, coating said granular material with a 45 foreign non-conductive substance, electrolytically depositing metal thereon, and subsequently removing said mold or core.

2. The galvanoplastic process which comprises applying to the surface of a mold or 50 core a coating of electrically conductive paint, coating said paint with grease and electrolytically depositing metal thereon.

3. The galvanoplastic process which comprises applying to the surface of an electrically non-conductive mold or core an 55 electrically conductive paint, coating said paint with a film of grease and subsequently electrolytically depositing metal thereon.

In testimony whereof I have signed my 60 name to this specification.

MATTHEW M. MERRITT.